

1

**3,184,311**  
**FURCELLARAN AS AN ANTISTATIC AGENT FOR**  
**PHOTOGRAPHIC FILM**

Wilho M. Salminen, Rochester, N.Y., assignor to Eastman Kodak Company, Rochester, N.Y., a corporation of New Jersey  
 No Drawing. Filed Mar. 9, 1962, Ser. No. 178,547  
 9 Claims. (Cl. 96—85)

This invention relates to photographic film, and more particularly to a film protected against static charges.

The accumulation of electrical charges on photographic film has been the cause of considerable difficulty in the past. In the ordinary handling operations, which occur in connection with the manufacture of sensitized photographic film, the film is passed over rollers, slides, and the like which result in the accumulation of static charges. When these static charges reach a sufficiently high intensity, a discharge can occur resulting in static lines on the sensitized film, which render the product unsuitable. Inasmuch as it is very difficult to determine whether films have been damaged by static charges until after it has been exposed and processed, it has been extremely desirable to protect the film from this accumulation.

Various methods have been used for protecting photographic film and paper against static charges by incorporating certain ionic organic materials including water soluble materials as described in Morey and White, U.S. 2,639,234. The use of water soluble inorganic acid salt has also been proposed. In addition, materials which absorb water and therefore provide a conductive surface have recently been employed. Most of these methods have not proven entirely satisfactory with the newer high-speed emulsions or with the different film types now being manufactured.

In addition to the requirements for static charge dissemination due to the conductivity of the antistatic agent, it is necessary to have a substance which is relatively inexpensive, which is effective in small amounts, and which is not detrimental to photographic emulsions.

We have found a material which can be used for protecting a sensitive photographic film against static charges and can also be incorporated in a photographic paper for the same purpose. This material is obtained from red alga and is known as furcellaran.

One object of this invention is to provide a novel and protective means of guarding against static. Another object is to provide a method of coating a photographic element in order to reduce its static tendency. A further object is to provide a suitable means for protecting cellulose acetate films, especially cellulose triacetate films against static. Still another object is to provide a means of producing photographic film of considerably lower electrical resistance while at the same time, retaining its optical transparency. Other objects will appear from the following descriptions of my invention:

The above objects are accomplished by coating photographic film base with furcellaran. This material forms a clear film, when coated as a 0.5-1.0% solution. This is coated on the film support at a preferred rate of about 120 milligrams per square foot. At least 50 milligrams per square foot is required, and it can be used as high as 1 gram per square foot.

Material may also be coated on photographic paper base in the same concentrations and may be incorporated in the photographic emulsion up to 50-100% based on the weight of the vehicle or coated on the reverse side of the support in the same concentrations of 50 milligrams to 1 gram per square foot.

Furcellaran is a potassium salt of the sulfuric ester of a high molecular weight polysaccharide. Typical analysis

2

reveals a polysaccharide content between 63 and 68%, the rest being essentially water plus potassium and calcium salts.

Furcellaran is commercially obtained from the red alga *Furcellaria fastigiata* which is found primarily in northern European waters, especially in the 600 square-mile area between Denmark and Sweden known as the Kattegat. The weed floats free and grows at depths of 20-30 feet. Trawlers collect the alga with nets, although some of the alga drifts on shore and is also collected for processing.

The furcellaran is extracted by setting the red alga out to bleach in the sun for three days after which it is preserved in lime for about three weeks. The material is then neutralized to remove impurities and to prepare the furcellaran in a soluble state for extraction.

The material is gelled and then frozen. When thawed, water and other impurities separate first leaving furcellaran behind. This product is then bleached and prepared for packaging.

The commercial furcellaran is a white odorless powder that is soluble in hot or warm water, forms gels at a low concentration and is extremely viscous; it is also relatively stable to heat.

The following examples are intended to illustrate my invention but not to limit it in any way:

*Example 1*

Two grams furcellaran is dissolved with stirring in 200 cc. hot water. A clear solution is formed. One cc. saponin solution (153.4 gms./1000 ccs. distilled water) is added as a coating aid. This is coated onto a subbed cellulose triacetate film support with a hand coater, at the rate of 120 milligrams of furcellaran per square foot.

*Example 2*

A dyed gelatin peloid is coated with a furcellaran anti-static coating as described in Example 1.

*Example 3*

A clear gelatin peloid is coated with a furcellaran coating as described in Example 1.

The following table shows the surface resistivity of the coated layers.

|                                     | Surface resistivity at<br>50% R.H., $10^{10}$ ohms |
|-------------------------------------|----------------------------------------------------|
| Results:                            |                                                    |
| Subbed film support                 | 10,000                                             |
| Dyed gelatin peloid                 | 21                                                 |
| Clear gelatin peloid                | 144                                                |
| Furcellaran on subbed film support  | .017                                               |
| Furcellaran on dyed gelatin peloid  | .091                                               |
| Furcellaran on clear gelatin peloid | .19                                                |

*Example 4*

Other polymeric films useful as film supports are coated with furcellaran at the rate of 100 milligrams per square foot. These film supports include polyethylene, polypropylene, cellulose acetate butyrate, cellulose acetate, cellulose nitrate, polyethylene terephthalate, and polystyrene. The resulting surface resistivities have an average value of  $0.025 \times 10^{10}$  ohms.

*Example 5*

Photographic paper is provided with an antistatic treatment by coating the paper with a concentration of 75 milligrams of furcellaran per square foot and is found to have an average surface resistivity of  $0.025 \times 10^{10}$  ohms. Satisfactory results are obtained by coating the furcellaran on the same side of the photographic paper as the photographic emulsion and also by coating the furcellaran on the reverse side of the paper.

3  
*Example 6*

Photographic paper having thereon a water-resistant coating is provided with an antistatic treatment by coating the paper with furcellaran in an amount of 1 gram per square foot. Satisfactory surface resistivities of less than  $10^{10}$  ohms are obtained when the coating is applied on the reverse side of the paper support and also when the coating is applied on the paper prior to applying over the coating the water-resistant polymeric coating. Satisfactory surface resistivities are also obtained by coating the furcellaran over the water-resistant coating layer. Polymeric coatings which are used to render the photographic paper water resistant include polystyrene, styrene-butadiene copolymers, vinylidenechloride-vinylchloride copolymers, polyethylene, polycarbonate, cellulose ester, and the like. Some of these polymeric coatings may require surface treatment such as electron bombardment, oxidation, and/or a subsequent subbing to obtain adhesion. However, these surface treatments or subbing coatings do not interfere with the effectiveness of the furcellaran coating as long as they are compatible with photographic emulsions.

The surfaces which are useful for carrying the photographic emulsion and which can be employed with furcellaran as an antistatic coating include those mentioned above as well as paper and the other polymeric materials which can be formed into suitable supports. These include polyesters, polycarbonates, polyolefins, polyacrylates, cellulose esters, cellulose ethers, and the like. Any type of polymeric material which can be used as a film support is operable in my invention, and the particular type of support is not critical.

Furcellaran can be coated on a film support on either side and is not removable during the processing steps so that it is a permanent antistatic layer. The use of a permanent antistatic layer of this type aids in protecting the film during its passage in the film handling mechanism in the camera itself. Moreover, after the film has been processed, particularly in connection with motion-picture film, the processed film has antistatic protection. This is particularly helpful in avoiding attraction to the film of dirt and dust particles which are picked up by charged motionpicture film supports.

The surface resistivity is measured by placing two parallel electrodes on the film at a fixed relative humidity of 50%; these electrodes are long compared to the distance between them so as to avoid end effects. The observed resistance reading is divided by the distance between electrodes and multiplied by their length to obtain the surface resistivity.

A surface resistivity below  $10^{10}$  ohms has been determined as a value which is sufficient to alleviate difficulties from static electricity generated in the normal handling of sensitive film. Furcellaran has an average surface resistivity of  $0.025 \times 10^{10}$  ohms which indicates its superior characteristics.

The invention has been described in considerable detail with particular reference to preferred embodiments thereof, but it will be understood that variations and modifications can be effected within the spirit and scope of the invention as described hereinabove and as defined in the appended claims.

4  
I claim:

1. A photographic film comprising a support having thereon a coating of furcellaran in an amount of 50 milligrams per square foot and also having thereon a light-sensitive silver halide emulsion layer to 1 gram per square foot.

2. A photographic film comprising a film support having thereon a coating of furcellaran, to impart antistatic properties thereto, in an amount of 50 milligrams to 1 gram per square foot and also having thereon a light sensitive silver halide emulsion layer.

3. A photographic paper comprising a paper base having thereon a coating of furcellaran in an amount of 50 milligrams per square foot and also having thereon a light-sensitive silver halide emulsion layer to 1 gram per square foot.

4. A photographic film comprising a film support having thereon a coating of furcellaran in an amount of 50 milligrams per square foot and also having thereon a light-sensitive silver halide emulsion layer to 1 gram per square foot.

5. A photographic paper comprising a paper base having thereon a coating of furcellaran in an amount of 50 milligrams per square foot to 1 gram per square foot and having thereon a light sensitive silver halide emulsion layer.

6. A photographic film comprising a film support and having thereon a coating of furcellaran in an amount of 50 milligrams per square foot to 1 gram per square foot and also having thereon a light sensitive silver halide emulsion layer.

7. A photographic element comprising a support having a layer thereon of light-sensitive silver halide dispersed in a carrier, said layer containing 50-100%, based on the weight of the carrier, of furcellaran.

8. Photographic paper base having a layer thereon of light-sensitive silver halide dispersed in gelatin, said layer containing 50-100%, based on the weight of the gelatin, of furcellaran.

9. Photographic film base having a layer thereon of light-sensitive silver halide dispersed in gelatin, said layer containing 50-100%, based on the weight of the gelatin, of furcellaran.

45  
**References Cited by the Examiner**

## UNITED STATES PATENTS

|           |       |               |       |       |
|-----------|-------|---------------|-------|-------|
| 2,639,234 | 5/53  | Morey et al.  | ----- | 96-87 |
| 2,725,297 | 11/55 | Morey         | ----- | 96-87 |
| 3,053,662 | 9/62  | Mackey et al. | ----- | 96-87 |
| 3,085,009 | 4/63  | Chambers      | ----- | 96-84 |
| 3,085,010 | 4/63  | Chambers      | ----- | 96-84 |

55  
**OTHER REFERENCES**

Whistler: Industrial Gums, TP978W5, pages 159 and 160.

Economic Botany, vol. 13, No. 4, October-December 1959, pages 365-370.

60 NORMAN G. TORCHIN, Primary Examiner.

UNITED STATES PATENT OFFICE  
CERTIFICATE OF CORRECTION

Patent No. 3,184,311

May 18, 1965

Wilho M. Salminen

It is hereby certified that error appears in the above numbered patent requiring correction and that the said Letters Patent should read as corrected below.

Column 4, lines 4, 14 and 19, after "foot", each occurrence, insert -- to 1 gram per square foot --; same column 4, lines 5 and 6, 15 and 16 and lines 20 and 21, strike out "to 1 gram per square foot", each occurrence.

Signed and sealed this 21st day of December 1965.

SEAL)

Attest:

ERNEST W. SWIDER

Attesting Officer

EDWARD J. BRENNER

Commissioner of Patents